

1

2,867,081

HYDROCARBON FUEL COMPOSITION AND THE  
METHOD OF OPERATING A JET ENGINE  
THEREWITHEllsworth E. Kimmel, Pittsburgh, Pa., assignor to Koppers  
Company, Inc., a corporation of DelawareNo Drawing. Application June 7, 1956  
Serial No. 589,861

19 Claims. (Cl. 60—35.4)

This invention relates to power plants of the type known as jet engines, their operation and hydrocarbon fuel compositions therefor. More particularly this invention relates to improved hydrocarbon fuel compositions for jet engines and the improved method of operation resulting therefrom. In one of its more specific aspects the invention relates to improved fuels for ram jet engines.

Currently there are three types of jet engines falling into categories known as turbo jets, ram jets, and pulse jets. The least complicated of these power plants is the ram jet engine. While it is similar in operation to the turbo jet with respect to its working cycle, the two engines differ in compression steps. Whereas compression for the turbo jet engine is provided by a gas turbine driven compressor which provides a stream of air to the combustion chamber at a desired controlled velocity, air flow through the combustion chamber of the ram jet engine is controlled only by the speed of the ram jet engine moving through the air. Compression for the ram jet engine is produced by the ramming effect of the oncoming air.

Heretofore operational difficulties encountered with jet engines were believed to be primarily due to engine design and the greatest effort was exerted in the development of better designs for jet engines capable of overcoming these difficulties. More recently, however, it has been found that not all hydrocarbons have the same characteristics when used as fuels in jet engines and that they differ in their burning characteristics sufficiently to cause notable differences in operation of jet engines.

One of the principal objectives in the development of ram jet engines is to provide a design which develops sufficient thrust to extend the present level to flight speed. Other important objectives are better fuel utilization, efficiency of fuel utilization being a function of speed of flight, and motor weight reduction. The thermal efficiency of ram jet engines operating at current flight levels is approximately 40%. Lower ignition temperatures and extended fuel to air ratio limits are to a great extent properties required in a fuel to reach these objectives.

One of the primary objects of this invention is to provide a fuel capable of developing a higher percentage increase in thermal efficiency at present flight speed levels and greater thrust for a given motor design.

Another important object of this invention is to provide hydrocarbon fuel compositions for jet engines having lower ignition temperatures.

Still another object of this invention is to provide a fuel capable of use under extended fuel to air ratio limits and having higher heats of combustion than fuels now available.

A still further object is to provide a new and novel igniter for hydrocarbon fuels and a new method of ignition.

The over-all search for fuel compositions capable of giving the optimum in engine operation has centered about additives whose properties in the combustion

2

process give (1) high heat of combustion, (2) high flame speed and having (3) high density, (4) low toxicity and (5) low volatility.

Unexpectedly, it now has been found that hydrocarbon fuel compositions eminently suitable for jet engines having certain of the most highly desired characteristics are made possible by utilization of the novel additives of this invention. Broadly speaking, in one aspect, invention resides in novel hydrocarbon fuel compositions containing as additives varying percentages of certain aluminum compounds more commonly known as aluminum alkyls. These compounds may be represented by the formula  $(R)_nAlH_{3-n}$  wherein R is a hydrocarbon radical and n is an integer of 1, 2 or 3.

Illustrative, but not limitative, of the aluminum alkyl additives which may be employed to advantage in the fuel compositions of this invention are trimethyl aluminum, dimethyl aluminum hydride, methyl aluminum dihydride, triethyl aluminum, diethyl aluminum hydride, ethyl aluminum dihydride, tributyl aluminum, dibutyl aluminum hydride, butyl aluminum dihydride, tri-isobutyl aluminum, di-isobutyl aluminum, isobutyl aluminum dihydride, and higher homologous aluminum alkyls and their hydrides.

In another embodiment of this invention it has been found that the additives above-described are very useful as igniters for hydrocarbon fuels, particularly in jet engine operation. When used in this manner, a small quantity of the aluminum alkyl is injected into the combustion zone of the engine where it contacts a pre-heated normally liquid hydrocarbon, causing the hydrocarbon to ignite. In addition to being useful for initial or start-up ignition, the aluminum alkyls can be used to reignite the fuel if "blow out" or "cut out" occurs.

In the first embodiment of this invention, the selected additive may be incorporated in the hydrocarbon fuel in a concentration ranging from about 5 to 30% by weight with about 5 to 10% being preferred.

When used as additives, the aluminum alkyls of this invention permit the use of a wide range of hydrocarbons such as conventional petroleum hydrocarbon jet engine fuels including kerosene and aviation gasoline. Generally hydrocarbon fractions which may be employed boil in the range of 200 to 700° F. A preferred fuel in accordance with this invention comprises a hydrocarbon fraction boiling in the range of 250 to 600° F. and containing the above-designated portions of an aluminum alkyl.

The fuels disclosed herein can be used in continuous type jet engines of the class known as turbo jet, ram jet, and pulse jet in which an atomizing type system for supplying fuel to the combustion chamber of the engine is employed. Generally these engines are operated by injecting the fuel and air into the combustion chamber of a jet engine in certain predetermined fuel-air ratios and igniting the fuel so as to heat the air and combustion gases, thus increasing the volume of gas mass which is exhausted through the exhaust zone of the jet engine. The exit of the gas mass from the rearwardly extending exhaust duct or jet nozzle is at a velocity higher than the flying speed of the engine. The thrust produced thereby equals the gas mass flowing through the exhaust duct times its increase in speed, according to the law of momentum.

In order to illustrate the advantages inherent in the hydrocarbon fuel compositions of this invention certain tests were performed to illustrate the temperatures at which the fuel compositions would ignite spontaneously in air and to illustrate the upper and lower limits of the fuel to air ratio outside of which combustion could no longer be supported. The point at which combustion will no longer be sustained is known as the "blow out" or "cut out" point. For comparison the same tests were

performed on hydrocarbons having no additive for the purpose of showing the advantages in the claimed compositions.

In order that those skilled in the art may have a fuller appreciation of the present invention the following examples are given by way of illustration and not by way of limitation. All parts and percentages are by weight unless otherwise specified.

#### IGNITION TESTS

##### Example I

Ignition tests were performed on a gasoline having the designation JP4 with no additive and on a 10% blend of tri-isobutyl aluminum in JP4. In the ignition tests, air was blown into a section of pipe approximately 8 feet long having an inside diameter of 14 inches. Gasoline was fed to this section of pipe at a controlled flow rate and burned in the air stream to preheat it. The air stream temperature was controlled by the quantity of gasoline burned in the air stream. Hot gases from the preheating section were passed through another section of pipe of the same length and diameter and then into a 4 foot section of pipe of the same diameter fitted with a multiplicity of nozzles for injecting fuel. The nozzles were uniformly distributed throughout a 6 inch length of this section. Contiguous to this section over a distance of about 1 foot the pipe was reduced from a 14 inch diameter to a 6 inch rectangular section having a single nozzle for the injection of fuel in ignition tests. From this section the gases were passed into another section of 14 inches inside diameter and then to the cooling section. The temperature of the air stream was gradually raised until ignition occurred. Evidence of ignition was a blue flame at the injection nozzle. The following results were obtained:

| Fuel                             | Ignition temperature          |
|----------------------------------|-------------------------------|
| JP4                              | Failed to ignite at 1,800° F. |
| 10% tri-isobutyl aluminum in JP4 | 800-1,000° F.                 |

The foregoing is clear evidence of a substantial improvement in ignition conditions as a direct result of employing the additives of the invention. More specifically, the decrease in ignition temperature is of the order of 800 to 1000° F.

Substitution of blends having 5 to 30% by weight of several of the aluminum alkyls listed above, for example triethyl aluminum, di-isobutyl aluminum monohydride and diethyl aluminum hydride gives ignition temperatures substantially lower than 1800° F. From these representative results it will be obvious to those skilled in the art that other aluminum alkyls and their hydrides can be used to advantage to lower hydrocarbon ignition temperatures. Triethyl aluminum, diethyl aluminum monohydride, tri-isobutyl aluminum and di-isobutyl aluminum monohydride have been found very effective for this purpose.

#### COMBUSTION TESTS

##### Example II

In the rectangular portion of the equipment described above were inserted flame stabilizers of the type employed in combustion tests. The purpose of these tests was to determine the upper and lower limits of the fuel to air ratio outside of which a flame or combustion could not be supported. The air velocity was 200 feet per second and it was preheated to 1000° F. In order to determine the lean limits after a steady flame had been achieved the fuel feed rate was decreased over a period of 10 to 15 seconds until the flame went out. To determine the rich limit, the fuel feed rate was gradually increased until the flame went out. In the following table are given the results of the combustion tests.

| Fuel                             | Fuel flow, gallons per hour |              |
|----------------------------------|-----------------------------|--------------|
|                                  | Lean mixture                | Rich mixture |
| JP4                              | 50                          | 140-145      |
| 10% tri-isobutyl aluminum in JP4 | 60                          | 165          |
| 10% triethyl aluminum in JP4     | 60                          | 185          |

In the foregoing combustion tests the fuel flows given are those flows at which the flame blew out. Each value given is the average of 3 to 4 determinations.

In additional combustion tests, 10 and 20% blends of triethyl aluminum in JP4 were tested in a 2 inch diameter, fuel atomizing type combustion chamber. In each case the blends burned under conditions where JP4 went out.

The foregoing ignition and combustion test results make it clear that substantially lower ignition temperatures are exhibited by the fuel compositions of the invention than the same fuel without additive, and that the low ignition temperature is also indicative of superior combustion properties.

While an air velocity of 200 feet per second was employed, further tests have shown that a higher air velocity of 500 to 600 feet per second gives even superior results.

The foregoing also clearly illustrates that by using alkyl aluminum in hydrocarbon fuels in accordance with this invention, extension of the rich fuel ratio is obtained which is equivalent to obtaining greater thrust for a given motor design. The amount of thrust is proportional to the quantity of fuel that can be consumed per unit of time. Extension of the upper level of fuel ratio, without flame "blow out" results in greater thrust. Similarly, it would be anticipated that for a given motor, addition of aluminum alkyls to the hydrocarbon would permit higher altitude flight limits as a result of extension of the rich fuel ratio.

As mentioned previously, the aluminum alkyls, in another aspect of this invention, are very useful for initial or start-up ignition or for reigniting following "blow out." Whereas ignition times in the neighborhood of 20 milliseconds is considered excellent, each of the aluminum alkyls tested in accordance with the invention gave ignition times of the order of 10 milliseconds. Specific ones of the aluminum alkyls which have given such reduced ignition times include triethyl aluminum, tri-isobutyl aluminum, diethyl aluminum hydride and di-isobutyl aluminum hydride. These tests were performed under normal operating conditions with a small quantity of the igniter being injected into the combustion zone of an engine containing the preheated fuel-air mixture and the ignition time recorded.

Various modifications of this invention will be apparent to those skilled in the art. It will also be obvious to those skilled in the art that alkyl aluminum other than those illustrated and of the class enumerated above and their hydrides can be employed to advantage in this invention. Such modifications are believed to be within the spirit and scope of this invention.

I claim:

1. The method of operating a jet engine which comprises supplying to the combustion zone of said jet engine a hydrocarbon fuel boiling in the range of 200° to 700° F. containing between 5 and 30% by weight of an aluminum compound having the formula  $(R)_nAlH_{3-n}$  wherein R is a lower alkyl radical and n is an integer equal to from 1 to 3, burning said fuel in the combustion zone of said engine and exhausting resulting gases from said engine so as to impart thrust thereto.

2. The method of claim 1 in which the aluminum alkyl is tri-isobutyl aluminum.

3. The method of claim 1 in which the aluminum alkyl is di-isobutyl aluminum monohydride.

4. The method of claim 1 in which the aluminum alkyl is triethyl aluminum.

5. The method of claim 1 in which the aluminum alkyl is diethyl aluminum monohydride.

6. The method of claim 1 in which the aluminum alkyl is trimethyl aluminum.

7. The method of igniting a jet fuel which comprises injecting an aluminum compound having the formula  $(R)_nAlH_{3-n}$  wherein R is a lower alkyl radical and n is an integer equal to from 1 to 3 into the combustion zone of a jet engine containing a normally liquid hydrocarbon boiling in the range of 200° to 700° F. and pre-heated to a temperature of about 800° to 1000° F.; said aluminum compound being introduced in an amount equal to from about 5% to 30% by weight of said hydrocarbon.

8. The method of claim 7 in which the aluminum compound is tri-isobutyl aluminum.

9. The method of claim 7 in which the aluminum compound is di-isobutyl aluminum monohydride.

10. The method of claim 7 in which the aluminum compound is triethyl aluminum.

11. The method of claim 7 in which the aluminum compound is diethyl aluminum monohydride.

12. The method of claim 7 in which the aluminum compound is trimethyl aluminum.

13. A jet engine fuel consisting essentially of a normally liquid hydrocarbon boiling in the range of 200° to 700° F. and about 5% to 30% by weight of an aluminum compound having the formula  $(R)_nAlH_{3-n}$  wherein R is a lower alkyl radical and n is an integer equal to from 1 to 3.

14. The jet engine fuel of claim 13 in which the aluminum alkyl is tri-isobutyl aluminum.

15. The jet engine fuel of claim 13 in which the aluminum alkyl is di-isobutyl aluminum monohydride.

16. The jet engine fuel of claim 13 in which the aluminum alkyl is triethyl aluminum.

17. The jet engine fuel of claim 13 in which the aluminum alkyl is diethyl aluminum monohydride.

18. The jet engine fuel of claim 13 in which the aluminum alkyl is trimethyl aluminum.

19. The method of operating a ram jet engine which comprises supplying to the combustion zone thereof a hydrocarbon fuel igniting in the range of about 800° to 1000° F. and boiling in the range of 250° to 600° F. containing between about 5% and 10% by weight of an aluminum compound having the formula:  $(R)_nAlH_{3-n}$  wherein R is a lower alkyl radical and n is an integer of at least one and not more than three, burning said fuel in the combustion zone of said jet engine and exhausting the resulting gases from said engine so as to impart thrust thereto.

#### References Cited in the file of this patent

#### UNITED STATES PATENTS

|           |                      |              |
|-----------|----------------------|--------------|
| 2,698,510 | Britton et al. ----- | Jan. 4, 1955 |
| 2,765,329 | Lindsey -----        | Oct. 2, 1956 |
| 2,775,863 | Traverse -----       | Jan. 1, 1957 |

#### OTHER REFERENCES

Chem. and Eng. News, vol. 26, No. 26, Sept. 27, 1948, pp. 2892-3.